

## UNITED STATES PATENT OFFICE

2,352,409

## MERCERIZING ASSISTANT

Hillary Robinette, Jr., Arlington, Mass., assignor to Commercial Solvents Corporation, Terre Haute, Ind., a corporation of Maryland

No Drawing. Application June 25, 1942,  
Serial No. 448,438

6 Claims. (Cl. 8—127)

My invention relates to the art of treating cotton fibers and fabrics. More particularly, it is concerned with the preparation of improved mercerizing baths, and a process for the treatment of cotton fibers and fabrics therewith.

In the initial processing of unkiered cotton yarn, unkiered piece goods, and kiered piece goods, it is necessary to subject the same to a mercerization treatment which involves the immersion of the yarn or goods in a caustic soda solution ranging in concentration of from about 18 to 30 per cent caustic. The purpose of this operation is generally three-fold, to-wit: it tends to strengthen the fibers, renders them more receptive of dyes, and imparts luster to the fibres. In order that the mercerization step be made use of to the fullest extent, however, it becomes necessary to add to the caustic, or mercerizing solution, a material known as a mercerizing assistant. In fact, with unkiered dry cotton, the presence of a mercerizing assistant in the mercerizing bath, is imperative. Otherwise, such cotton cannot be wetted by caustic solutions of mercerizing strength. In general, the use of a mercerizing assistant, if efficient, insures even penetration of the caustic and uniform luster of the material thus treated.

Previously, attempts have been made to improve the wetting and penetrating properties of mercerizing baths, by adding thereto numerous materials of a widely varying character, such as, for example, soaps, Turkey red oils, sulfonated fats, aromatic sulfonic acids, as well as phenol, and its homologs, with or without addition of special solvents, such as aliphatic or aromatic alcohols. Because of the tendency to be salted out on account of the high electrolyte content of the caustic soda contained in the mercerizing bath, some of these agents were found to either be usable only for a short time, or to be impractical under any conditions. Some of the solvents employed volatilize in a short time, or under certain conditions are found to be only difficultly soluble in the mercerizing bath, and, as a result, small particles thereof coalesce into large globules which float on top of the bath, adhere to the fibers, and interfere with the uniform impregnation of the fibrous material with the caustic soda.

I have now discovered that highly satisfactory mercerizing baths possessing none of the aforesaid disadvantages, may be prepared by adding to a caustic solution of mercerizing strength, a relatively small quantity of 2-methyl-2,4-pentanediol, together with a sufficient volume of a

phenolic type compound (solubilizing agent) to render the 2-methyl-2,4-pentanediol soluble in the mercerizing bath. The amount of 2-methyl-2,4-pentanediol employed may vary from between about 10 and 30 per cent by weight of the solubilizing agent utilized, while the total amount of solubilizing agent and 2-methyl-2,4-pentanediol that may be used in preparing mercerizing baths of the above-mentioned type, can vary from between approximately 0.35 to 2.0 per cent by volume of the mercerizing bath. In general, it will be observed that for mercerizing baths of decreasing alkalinity, a correspondingly increased amount of my mercerizing assistant should be added. However, for mercerizing baths of any given alkalinity, the amount of mercerizing assistant necessary to give optimum results, may be readily established by simple experiment.

As examples of suitable solubilizing agents, there may be mentioned phenol, ortho-, meta-, and para-cresols, cresylic acid, xylenols, mixtures of the cresols and xylenols, the monochloro- and monobromo-phenols and cresols, carvacrol, and the like, and mixtures that are derivable from the above-mentioned types of compounds.

The advantages of mercerizing assistants of the type covered by the present invention over those previously utilized, are many. For example, such mercerizing assistants are designed to perform effectively in substantially any given concentration of caustic solution suitable for mercerizing operations. They insure the even penetration of caustic into the yarn or fabric being mercerized, thus giving higher luster and even dyeing properties to the mercerized yarn or fabric, and, as a result, eliminate the possibility of having yarn or piece goods rejected because of uneven dyeing thereof. Also, by the use of my mercerizing assistants, the time ordinarily required in the mercerization of cotton, is materially reduced. A further economical advantage is the fact that by employing the present invention, it is possible to reduce the caustic content of the mercerization bath, and still obtain satisfactory results. Other additional advantages of my mercerizing assistants are that they insure the uniform tensile strength of the mercerized yarn or fabric, and all of said mercerizing assistants can be dissolved directly in the mercerizing bath. Further advantages of these mercerizing assistants lie in the fact that the necessity of any pretreatment of the material to be mercerized is eliminated, and that they are capable of being readily removed from the mercerized cloth in subsequent scouring operations.

One of the most unpredictable and surprising features of my invention is the fact that I have found, out of numerous glycols tested, only 2-methyl-2,4-pentanediol to be of any practical value as a mercerizing assistant; even hexamethylene glycol, an isomer of 2-methyl-2,4-pentanediol, proved to be unsatisfactory when employed in accordance with my invention.

In obtaining the data presented below, the various mercerizing assistants were added in the amounts indicated, to a 25 per cent sodium hydroxide solution. The wetting-out test employed consisted of dropping a small bundle containing 120 ends of 1-inch lengths of unbleached cotton yarn on the surface of the solution of mercerizing assistant in caustic. The number of seconds required for the bundle to wet completely and sink below the surface, was then noted.

Shrinkage determinations were carried out by first placing 50 cc. of caustic solution containing a known amount of mercerizing assistant in a 50 cc. graduated cylinder. A small steel weight was then tied to one end of a piece of 4-ply unboiled cotton yarn, while the other end was drawn through a notched rubber stopper of a size to fit the top of the glass graduate. The length of the string from the weight to the stopper was then adjusted so that the weight just barely touched the bottom of the cylinder. The weighted string was next dropped into the caustic solution, and the degree of shrinkage in 20 seconds was measured by noting the rise of the weight from the bottom of the graduated cylinder. The shrinkage tests, as well as the wetting-out tests, were determined at room temperature.

The following table shows the composition of the various mercerizing assistants used, and summarizes the results obtained in accordance with the procedures outlined generally above:

| Mercerizing assistant            | Per cent added to mercerizing bath | Wetting out time | Per cent shrinkage |
|----------------------------------|------------------------------------|------------------|--------------------|
| 18 g. cresylic acid.             | 0.50                               | 3 sec.....       | 15.4               |
| 5.3 g. 2-methyl-2,4-pentanediol. | 0.50                               | 3 sec.....       | 16.6               |
| 4 g. cresylic acid.              | 0.50                               | 9 sec.....       | 12.2               |
| 18 g. cresylic acid.             | 0.50                               | 12 sec.....      | 12.2               |
| 1.8 g. 2-methyl-2,4-pentanediol. | 0.50                               | Over 2 min..     | 2.2                |
| 18 g. cresylic acid.             | 0.50                               | Over 2 min..     | 2.2                |
| 2 g. ethylene glycol.            | 0.50                               | Over 2 min..     | 2.2                |
| 18 g. cresylic acid.             | 0.50                               | Over 2 min..     | 2.2                |
| 2 g. trimethylene glycol.        | 0.50                               | Over 2 min..     | 2.2                |
| 18 g. cresylic acid.             | 0.50                               | Over 2 min..     | 2.2                |
| 2 g. propylene glycol.           | 0.50                               | Over 2 min..     | 2.2                |
| 18 g. cresylic acid.             | 0.50                               | Over 2 min..     | 2.2                |
| 2 g. glycerine.                  | 0.50                               | Over 2 min..     | 1.1                |
| 18 g. cresylic acid.             | 0.50                               | Over 2 min..     | 4.5                |
| 2 g. 2,3-butylene glycol.        | 0.50                               | Over 2 min..     | 1.1                |
| 18 g. cresylic acid.             | 0.50                               | Over 2 min..     | 1.1                |
| 4 g. hexamethylene glycol.       | 1.00                               | Over 2 min..     | 1.1                |
| Cresylic acid.                   |                                    |                  |                    |

It is to be understood that the data appearing

above are merely illustrative of my process, and are to be in no way considered limitative. In general, it may be said that the results shown in the above table may be duplicated by adding the required amount of 2-methyl-2,4-pentanediol to a caustic solution of mercerizing strength which contains a solubilizing agent capable of dissolving the 2-methyl-2,4-pentanediol in said caustic solution. It is to be further understood that the term "solubilizing agent" appearing in certain of the appended claims, is to be construed to include any solubilizing agents having the aforesaid properties.

Having described my invention, what I claim is:

1. A mercerizing assistant suitable for addition to an alkaline mercerizing bath, said assistant comprising essentially 2 - methyl - 2,4-pentanediol and a solubilizing agent selected from the group consisting of phenol, ortho-, meta-, and para-cresols, cresylic acid, xlenols, mixtures of the cresols and the xlenols, monochloro- and monobromo-phenols and cresols, and carvacrol.
2. A mercerizing assistant suitable for addition to an alkaline mercerizing bath, said assistant comprising essentially cresylic acid and 2-methyl-2,4-pentanediol.
3. A process for increasing the wetting and penetrative capacity of alkaline mercerizing baths, which consists of adding to the mercerizing bath 2-methyl-2,4-pentanediol and a solubilizing agent selected from the group consisting of phenol, ortho-, meta-, and para-cresols, cresylic acid, xlenols, mixtures of the cresols and the xlenols, monochloro- and monobromo-phenols and cresols, and carvacrol.
4. A process for increasing the wetting and penetrative capacity of alkaline mercerizing baths, which consists of adding to the said mercerizing bath cresylic acid and 2-methyl-2,4-pentanediol.
5. A process for increasing the wetting and penetrative capacity of alkaline mercerizing baths, which consists of adding from between about 0.35 to 2.0 per cent of a mixture comprising essentially 2-methyl-2,4-pentanediol and a solubilizing agent selected from the group consisting of phenol, ortho-, meta-, and para-cresols, cresylic acid, xlenols, mixtures of the cresols and the xlenols, monochloro- and monobromo-phenols and cresols, and carvacrol.
6. A process for increasing the wetting and penetrative capacity of alkaline mercerizing baths, which consists of adding from between about 0.35 and 2.0 per cent of a mixture comprising essentially cresylic acid and 2-methyl-2,4-pentanediol.

HILLARY ROBINETTE, JR.